

## UNITED STATES PATENT OFFICE

2,161,763

## PROCESS OF MAKING PAPER PULP

Edwin P. Jones, Garden City, N. Y., assignor to  
 Champagne Paper Corporation, New York,  
 N. Y., a corporation of New York

No Drawing. Application October 6, 1937,  
 Serial No. 167,582

1 Claim. (Cl. 92—13)

The present invention relates to the production of high grade paper stock from straw of the nature of flax and hemp.

A feature of the present invention is an improved method of treating straw of the nature of flax straw in such a manner as to facilitate the removal of ligneous and incrusting constituents thereof, and thereby facilitate the subsequent bleaching of the resulting paper stock.

10 The invention is applicable in processing straw of the nature of flax straw and particularly flax which is raised primarily for the seed rather than for the fiber. Such flax straw is difficult to process in that the seed flax straw is allowed to mature 15 in the fields and this fact renders the same more difficult to process than tow produced from fiber flax straw which does not fully mature before harvesting. Paper stock produced from seed flax straw is particularly difficult to bleach.

20 According to the present invention the flax straw or other straw of the nature of flax straw is de-seeded and preferably broken advantageously by the employment of a conventional type of flax brake which is employed for de-seeding and 25 breaking the straw in one operation with a resultant minimum loss of fiber.

The crude fiber or tow resulting from the breaking operation is then subjected to a predigestion operation in the presence of water at a steam 30 pressure ranging from 60 to 80 pounds per square inch and preferably approximately 75 pounds per square inch for a period of time of approximately 35 25 to 40 minutes. This treatment has been found to be efficacious in removing certain substances which cement or bind the fiber to the woody portion of the tow, as inspection of the predigested material discloses that the fibers are less tightly bound to this woody portion. This effect cannot 40 be produced by the mere immersion of the tow in water as has heretofore been done.

The tow resulting from the predigestion operation is then subjected to the action of a suitable agent, primarily for the treatment of the ligneous and incrusting constituents present therein. This 45 step is carried out effectively by an aqueous solution of, or yielding sodium hydroxide and sulphur, at suitable temperatures and preferably in a pressure cooker or digester.

50 Excellent results have been obtained by an aqueous solution of sodium hydroxide and sulphur, and in my present invention I effect a marked saving in the amount of chemicals used over that heretofore employed.

55 The predigested tow resulting from the digestion of the tow in the presence of water at a steam pressure of from 60 pounds to 80 pounds per

square inch, for from 25 to 40 minutes may be subjected to a digestion operation with a mixture of sodium hydroxide and sulphur in the presence of water with a substantial saving of chemicals. While not definitely established, this saving of 5 chemicals is probably the result of two factors:

(a) The predigestion operation is undoubtedly instrumental in causing the removal of more substances than is caused by mere immersion of tow in water at or near room temperature. 10

(b) The predigested tow does not absorb or retain so much water as does tow which is simply immersed in water at or near room temperature. As a result it has been found practical to cook the predigested material with less water than is usually used in the case of water immersed tow. 15 This means that less chemical is required because the concentration of the chemicals as determined by the amount of water and chemicals present is one of the determining factors in the cooking 20 operation.

While the predigestion operation has associated with it certain disadvantages, as for example, additional steam is used in the predigestion operation and in commercial practice some time is 25 required to heat the digester and contents to the pressure required, and to allow the digester and contents to cool, yet it is estimated that the saving in chemicals effected by the predigestion operation more than offsets the disadvantages set out 30 above, and in addition the resulting product is measurably superior to any which has heretofore been produced by known methods.

While relatively specific proportions, with regard to pressures and time employed have been 35 set out in this specification, yet it is to be understood such proportions may be varied within relatively wide limits without departing from the spirit of the invention.

I claim:

That improved method of producing bleached pulp from flax or hemp tow, which consists in subjecting the tow to a predigestion operation in the presence of water at a steam pressure of from 60 to 80 pounds per square inch for from 25 to 40 minutes, then washing the tow, then subjecting the tow to a cooking operation in a digester with a solution of water of approximately 2 to 4 times the dry weight of the fiber, and 10 percent to 20 percent sodium hydroxide, and one-half to four percent sulphur, the quantities of the chemicals employed in the solution being based on the dry weight of the tow, then washing the cooked fiber to remove water soluble impurities, and bleaching 50 the washed pulp. 45

EDWIN P. JONES. 55